

## UNITED STATES PATENT OFFICE

1,959,316

DISTILLATE PETROLEUM PRODUCT AND  
METHOD OF TREATING SAME

James B. Rather, Brooklyn, Orland M. Reiff,  
Jackson Heights, and Leslie C. Beard, Jr.,  
Brooklyn, N. Y., assignors to Socony-Vacuum  
Corporation, New York, N. Y., a corporation of  
New York

No Drawing. Application September 25, 1929,  
Serial No. 395,192

16 Claims. (Cl. 44—9)

This invention relates to distillate petroleum products, more particularly gasoline and kerosene, and to a method of and means for imparting a stability thereto with respect to color, 5 gum formation and odor, and for removing any objectionable color developed therein during storage.

Heretofore we have discovered that certain organic compounds of the nature of negative oxidation catalysts have the property of preventing or materially delaying the formation of color, gum and malodorous constituents in distillate petroleum products, particularly gasoline and kerosene. Notable amongst these compounds are 15 the hydroxybenzenes, especially hydroquinone and pyrogallol. Certain of these compounds, particularly hydroquinone and pyrogallol, have the added property of decolorizing distillate petroleum products which have become discolored 20 during storage.

We have found, however, that a number of these compounds will not function properly in the presence of water, due to the fact that they are considerably more soluble in water than in the 25 distillate petroleum products. This characteristic materially affects the commercial value of these compounds as stabilizers and decolorizers, particularly when the treated distillates are handled in bulk, because of the difficulties involved 30 in maintaining tankers, storage tanks, pipe lines and delivery trucks free of water.

In accordance with the present invention, however, the decolorization and/or the stabilization 35 of distillate petroleum products with regard to color, gum formation and odor may be readily and effectually attained regardless of the presence of water, by the use of certain water insoluble compounds we have found to be suitable for the purpose.

40 One of the objects of the present invention is to provide a method of and means for effectually decolorizing and/or stabilizing distillate petroleum products with respect to color, gum formation and odor in the presence of water.

45 Another object of the invention is to provide agents or compounds which in the presence of water, will effectually decolorize and/or stabilize distillate petroleum products with respect to color, gum and odor.

50 Another object of the invention is to provide water insoluble agents or compounds which are effective as decolorizers and/or stabilizers of distillate petroleum products with respect to color, gum formation and odor.

55 Another object of the invention is to provide

agents or compounds effective in removing initial or recurrent discoloration of distillate petroleum products and for stabilizing the same as to color, odor, and the formation of gum, which agents or compounds are soluble in the distillates 60 and insoluble in water.

A further object of the invention is to provide agents or compounds of the character referred to which are unaffected in their action by the presence of water.

65 Other objects of the invention will be apparent from the following description.

Among the compounds in the nature of negative oxidation catalysts that we have discovered are suitable for the objects set forth are the 70 alkyl substituted hydroxybenzenes, such as the diamyl and methyl substituted hydroxybenzenes, particularly diamyl hydroquinone and tolu hydroquinone. These compounds are formed preferably by substituting alkyl groups for some of 75 the hydrogens in hydroxybenzenes such as hydroquinone and are substantially insoluble in water but readily soluble in distillate petroleum products. For example, diamyl hydroquinone

80  $[(C_5H_{11})_2C_6H_2(OH)_2]$

is soluble in distillate petroleum products, such as kerosene, to the extent of one part of diamyl hydroquinone to approximately eight hundred parts 85 of kerosene and is practically insoluble in water. Hydroquinone, on the other hand, is not as soluble in petroleum distillates, being soluble to the extent of one part of hydroquinone to approximately one hundred thousand parts of kerosene while it readily dissolves in water to the extent 90 of approximately six parts of hydroquinone to one hundred parts of water.

A relatively minute amount, preferably less than 0.01% of the agent or compound may be thoroughly mixed with the distillate to be treated, 95 although it will be understood that the distillate may be percolated through a mass of the compound, if desired. Preferably, however, the compound is first dissolved in a suitable solvent which is miscible in the distillate, such as an aliphatic alcohol, particularly isopropyl alcohol, in the proportion of one part of the compound to approximately ten parts of the solvent. The resulting solution is then added to the distillate to be treated in minute amounts, preferably less than 0.1%. 105 This method usually results in the compound being distributed throughout and dissolved in the distillate more readily than if it were added directly thereto.

110 The results of the following tests will illustrate

the effectiveness of the treatment of distillate petroleum products in accordance with our invention. Samples of a kerosene which had developed a color of minus 15 Saybolt during storage 5 were treated with one part of compound to approximately 25,000 parts of the kerosene and after decolorization, each of the samples was contacted with 20% by volume of water and the color noted after periods of one day and one week. The 10 sample treated with diamyl hydroquinone after one day had a color of plus 13 and maintained this color to the time of the second reading at the end of a week. The sample treated with tolu hydroquinone had a Saybolt color after one day 15 of plus 13 and after a week, a color of plus 6.

Other samples were treated with hydroquinone and pyrogallol to obtain comparative data. The 20 sample treated with hydroquinone after one day had a color of plus 11 Saybolt and after one week, the color had changed to minus 5. The sample 25 treated with pyrogallol, after one day had a color of plus 10 and after a week, a color of plus 2.

Other samples, however, treated with hydroquinone and pyrogallol, in the absence of water 30 held their restored color of plus 11 and plus 10 respectively, as noted above, for several months without change.

Diamyl hydroquinone is prepared by condensing amylene with hydroquinone in the presence 35 of sulfuric and glacial acetic acids at ordinary temperatures, Koenig, Berichte 25, 2650 (1892).

While we have thus specifically described our 40 invention, various modifications thereof may suggest themselves to those skilled in the art, and it therefore is our intention that the invention 45 be limited only by the scope of the appended claims.

Having thus described our invention, what we 50 claim and desire to secure by Letters Patent is:

40 1. A petroleum distillate product capable of use as a motor fuel lying within the gasoline-kerosene range normally tending to deteriorate on storage by formation of varying relative proportions of gum and color stabilized by the addition of a small quantity of an alkyl substituted hydroquinone, the alkyl group being substituted for hydrogen of the benzene nucleus.

45 2. A petroleum distillate product capable of use as a motor fuel lying within the gasoline-kerosene range normally tending to deteriorate on storage by formation of varying relative proportions of gum and color stabilized by the addition of a small quantity of a diamyl substituted hydroquinone, the amyl group being substituted for hydrogen of the benzene nucleus.

50 3. A low boiling normally light colored distillate petroleum product of the class of gasoline or kerosene which normally tends to deteriorate by oxidation, as evidenced by the formation of color or gum therein during storage, having added thereto a small amount of an alkyl substituted dihydroxy benzene sufficient substantially to retard the aforesaid deterioration, the alkyl group being substituted for hydrogen of the benzene nucleus.

55 4. A low boiling normally light colored distillate petroleum product of the class of gasoline or kerosene which normally tends to deteriorate by oxidation, as evidenced by the formation of color or gum therein during storage, having added thereto a small amount of an alkyl substituted hydroquinone sufficient substantially to retard the aforesaid deterioration, the alkyl group being substituted for hydrogen of the benzene nucleus.

60 5. A low boiling normally light colored distillate

late petroleum product of the class of gasoline or kerosene which normally tends to deteriorate by oxidation, as evidenced by the formation of color or gum therein during storage, having added thereto a small amount of a diamyl substituted hydroquinone sufficient substantially to retard the aforesaid deterioration, the amyl group being substituted for hydrogen of the benzene nucleus.

65 6. A low boiling normally light colored distillate petroleum product of the class of gasoline or kerosene which normally tends to deteriorate by oxidation, as evidenced by the formation of color or gum therein during storage, having added thereto a small amount of a methyl substituted hydroquinone sufficient substantially to retard the aforesaid deterioration, the methyl group being substituted for hydrogen of the benzene nucleus.

70 7. A boiling normally light colored distillate petroleum product of the class of gasoline or kerosene which normally tends to deteriorate by oxidation, as evidenced by the formation of color or gum therein during storage, having added thereto a small amount of a diamyl substituted dihydroxy benzene sufficient substantially to retard the aforesaid deterioration, the amyl group being substituted for hydrogen of the benzene nucleus.

75 8. A low boiling normally light colored distillate petroleum product of the class of gasoline or kerosene which normally tends to deteriorate by oxidation, as evidenced by the formation of color or gum therein during storage, having added thereto a small amount of a methyl substituted dihydroxy benzene sufficient substantially to retard the aforesaid deterioration, the methyl group being substituted for hydrogen of the benzene nucleus.

80 9. The method of stabilizing the characteristics 85 of a low boiling normally light colored petroleum distillate product of the class of gasoline or kerosene that normally tends to deteriorate by oxidation, as evidenced by the formation of color or gum therein during storage, which comprises adding thereto, prior to substantial deterioration as aforesaid, a small proportion of an alkyl substituted dihydroxy benzene sufficient substantially to retard the aforesaid deterioration, the alkyl group being substituted for hydrogen of the benzene nucleus.

85 10. The method of stabilizing the characteristics 90 of a low boiling normally light colored petroleum distillate product of the class of gasoline or kerosene that normally tends to deteriorate by oxidation, as evidenced by the formation of color or gum therein during storage, which comprises adding thereto, prior to substantial deterioration as aforesaid, a small proportion of a diamyl substituted hydroquinone sufficient substantially to retard the aforesaid deterioration, the amyl group being substituted for hydrogen of the benzene nucleus.

95 11. The method of decolorizing a normally light colored low boiling petroleum distillate product 95 of the class of gasoline or kerosene which has become discolored by spontaneous color formation during storage, which comprises adding to said discolored product a small proportion of an alkyl substituted dihydroxy benzene sufficient to 100 effect removal of a substantial proportion of the aforesaid discoloration, the alkyl group being substituted for hydrogen of the benzene nucleus.

100 12. The method of decolorizing a normally light colored low boiling petroleum distillate product 100 of the class of gasoline or kerosene which has

- of the class of gasoline or kerosene which has become discolored by spontaneous color formation during storage, which comprises adding to said discolored product a small proportion of an alkyl substituted hydroquinone sufficient to effect removal of a substantial proportion of the aforesaid discoloration, the alkyl group being substituted for hydrogen of the benzene nucleus. 13. The method of decolorizing a normally light colored low boiling petroleum distillate product of the class of gasoline or kerosene which has become discolored by spontaneous color formation during storage, which comprises adding to said discolored product a small proportion of a diamyl substituted hydroquinone sufficient to effect removal of a substantial proportion of the aforesaid discoloration, the amyl group being substituted for hydrogen of the benzene nucleus. 14. The method of decolorizing a normally light colored low boiling petroleum distillate product of the class of gasoline or kerosene which has become discolored by spontaneous color formation during storage, which comprises adding to said discolored product a small proportion of a methyl substituted hydroquinone sufficient to effect removal of a substantial proportion of the aforesaid discoloration, the methyl group being substituted for hydrogen of the benzene nucleus. 15. The method of decolorizing a normally light colored low boiling petroleum distillate product of the class of gasoline or kerosene which has become discolored by spontaneous color formation during storage, which comprises adding to said discolored product a small proportion of a diamyl substituted dihydroxy benzene sufficient to effect removal of a substantial proportion of the aforesaid discoloration, the amyl group being substituted for hydrogen of the benzene nucleus. 16. The method of decolorizing a normally light colored low boiling petroleum distillate product of the class of gasoline or kerosene which has become discolored by spontaneous color formation during storage, which comprises adding to said discolored product a small proportion of a methyl substituted dihydroxy benzene sufficient to effect removal of a substantial proportion of the aforesaid discoloration, the methyl group being substituted for hydrogen of the benzene nucleus.
- 80 85 90 95
- JAMES B. RATHER.  
ORLAND M. REIFF. 100  
LESLIE C. BEARD, JR.
- 30 105
- 35 110
- 40 115
- 45 120
- 50 125
- 55 130
- 60 135
- 65 140
- 70 145
- 75 150